

[54] ADDITION AGENT FOR MOLTEN METALS  
AND PROCESS FOR MAKING THE SAME[76] Inventors: **Luigi Palumbo**, via Eusebio Chini  
22; **Raffaele Tarozzi**, via Marangoni  
N. 1, both of Rome, Italy[22] Filed: **June 20, 1974**[21] Appl. No.: **481,546**

## [30] Foreign Application Priority Data

June 20, 1973 Italy ..... 50929/73

[52] U.S. Cl. ..... **75/130; 75/53; 252/475;**  
264/117[51] Int. Cl.<sup>2</sup>. **C22C 33/08; B01J 23/02; C09C 1/56**[58] Field of Search ..... 75/53, 130; 252/475, 476;  
264/117

## [56] References Cited

## UNITED STATES PATENTS

2,881,068 4/1959 Bergh ..... 75/53  
3,656,989 4/1972 Layland ..... 75/130 RPrimary Examiner—Peter D. Rosenberg  
Attorney, Agent, or Firm—Young & Thompson

## [57] ABSTRACT

An addition agent for adding an alkali metal or alkaline earth metal to a molten metal bath, for example for the addition of magnesium to a molten iron bath in the production of nodular cast iron in which the graphite is spheroidal in the as-cast condition, comprises briquettes of 5-50 percent by weight of the inoculant metal of a particle size 0.1 to 3 mm., 50-80 percent by weight of a porous material such as semi-coke, coke or graphite, having a particle size of 0.1 to 3 mm., and 10-25 percent by weight of a binder such as coal-tar pitch, coal-tar, or petrochemical pitch or bitumen. The inoculant metal and porous material are first admixed and then homogenized with the binder at a temperature of 80-130°C., after which briquetting is conducted. The briquettes are then heated from 150-250°C. for 15 to 90 minutes to harden them, and may be further heated for that period of time at 250-990°C. to bake them.

7 Claims, No Drawings

ADDITION AGENT FOR MOLTEN METALS AND  
PROCESS FOR MAKING THE SAME

The present invention relates to addition agents for facilitating the addition of metals to molten metal baths, and to processes for the production of the same. More particularly, the present invention relates to such addition agents and processes, for the addition in a controlled manner to a molten metallic bath, of metals which are relatively volatile and/or easily oxidized and/or violently reactive with the metal bath.

For example, in the production of nodular cast iron, in which spheroidal graphite is produced in the as-cast form by the inoculation of the bath with small amounts of magnesium, a difficulty arises from the fact that the boiling point of magnesium is below the melting point of iron. Similar problems arise in steelmaking in connection with ladle desulfurization of the hot metal prior to refining.

In the past, a number of techniques and products for the inoculation of baths such as ferrous metal baths have been proposed, among them being the use of a porous support material as a vehicle for the inoculant metal. Such a porous support has been for example coke, impregnated with the desired metal in the molten state. Techniques for the production of such additives are disclosed for example in Italian Pat. Nos. 743,720 and 904,658, and comprise immersion of the porous material in the molten inoculant metal, followed by rapid cooling to solidify the metal which has penetrated the pores of the support.

However, such techniques and the resulting products have drawbacks by virtue of the high reactivity and temperature of the inoculant metal. Thus, carbides form by the partial reaction of the metal with the carbon of the coke, and these carbides in the presence of moisture react to emit flammable gases. Moreover, the surface mechanical properties of the finished product correspondingly deteriorate. If the cooling medium is oil, then this can ignite. The active metal can oxidize when the cooling medium contains oxygen; and nitrides can form when the cooling medium contains nitrogen.

Accordingly, it is an object of the present invention to provide an addition agent as defined above and a process for producing the same, which will overcome the foregoing difficulties and disadvantages.

Another object of the present invention is the provision of such addition agents which will be relatively simple and inexpensive to produce and reliable in result when used, and to provide such processes for the production thereof which will be easy to practice and dependable in result.

Briefly, the objects of the present invention are achieved by providing an addition agent and a process for producing the same, usable in various pyrometallurgical operations such as hot metal desulfurization and the nodularization of cast iron, in which particles of the reactive metal and particles of a porous material are admixed with each other and then with a binder, and then heated. The resulting product is uniform both dimensionally and compositionally and is not subject to the drawbacks and disadvantages recited above.

Further objects, features and advantages of the present invention will become apparent from a consideration of the following more detailed description of the invention.

In greater detail, the invention comprises the formation of a mixture consisting essentially of particles of the active material and particles of the porous support material which is then admixed with a binder, followed by briquetting of the mixture. The briquetted mixture is then heated. Thereafter, if required, the briquettes are baked.

The composition by weight of the product can be as follows:

|                 |        |
|-----------------|--------|
| Metal           | 5-50%  |
| Porous material | 50-80% |
| Binder          | 10-25% |

Homogenization and briquetting of the mixture can be conducted between 80° and 130°C. Subsequent heating of the briquettes takes place between 150° and 250° C. and for a time between 15 and 90 minutes. Baking of the briquettes, if carried out, can be performed at a temperature in a range of 250°-900°C. and for the same time period.

The metal may be alkali metal or alkaline earth metal, or in general, any metal which is added to a molten metal bath and which has, relative to the bath, great volatility and/or a high tendency toward oxidization and/or violent reactivity with the bath. Examples are sodium, potassium, magnesium, calcium and strontium. The metal may be in the form of pure metal or an alloy thereof. The particle size is between 0.1 and 3 mm.

The bath itself may be any of the molten metal baths encountered in pyrometallurgy, and will ordinarily be ferrous, e.g., iron, nickel, cobalt or an alloy thereof.

The porous material may be semi-coke, coke, graphite, or any similar compound or substance which has sufficient porosity and mechanical strength. The particle size may be 0.1 to 3 mm.

The binder may be coal tar pitch, coal tar, pitch or bitumen of petrochemical origin or mixtures of these in various proportions. Homogenization with the mixed particles of the active metal and the porous material is carried out for example in a masticator at a temperature between 80° and 130°C. but which ordinarily will not exceed by more than 50°C. the softening temperature of the binder.

To enable those skilled in this art to practice the invention, the following illustrative example is given:

A mixture is formed of 60 parts by weight of semi-coke of particle size from 0.3 to 1 mm. and 20 parts by weight of magnesium particles of particle size from 0.1 to 0.3 mm. It is admixed in a masticator with 20 parts by weight of coal tar pitch having a softening point of 43.5°C., at a temperature of 90°C. for 10 minutes. The mixture thus obtained was briquetted in a press to obtain spherical briquettes 32 mm. in diameter. The briquettes were then hardened by exposure for 30 minutes in a current of air at 200°C. with a flow rate of 150 N1/h. The hardened briquettes were then baked by exposure for 30 minutes in a current of hydrogen having a temperature of 700°C. and a flow rate of 150 N1/h. The briquettes obtained showed the following properties at various stages:

|                     | Density<br>g/cm <sup>3</sup> | Compressive<br>Strength<br>kg |
|---------------------|------------------------------|-------------------------------|
| Green briquettes    | 1.04                         | 80                            |
| Hardened briquettes | 1.03                         | 120                           |

-continued

|                  | Density<br>g/cm <sup>3</sup> | Compressive<br>Strength<br>kg |
|------------------|------------------------------|-------------------------------|
| Baked briquettes | 0.93                         | 300                           |

The yield after baking is 90 percent.

The briquetted addition agent thus obtained is useful in ferrous metallurgy as an addition agent for inoculating a bath of molten iron in a production of cast iron containing nodular or spheroidal graphite in the as-cast condition.

From a consideration of the foregoing disclosure, therefore, it will be evident that all of the initially recited objects of the present invention have been achieved.

Although the present invention has been described and illustrated in connection with preferred embodiments, it is to be understood that modifications and variations may be resorted to without departing from the spirit of the invention, as those skilled in this art will readily understand. Such modifications and variations are considered to be within the purview and scope of the present invention as defined by the appended claims.

Having described our invention we claim:

1. An addition agent for the inoculation of a molten metal bath, consisting essentially of 5 to 50 percent by weight of a metal selected from the group consisting of alkali metal and alkaline earth metal having a particle size 0.1 to 3 mm., 50 to 80 percent by weight of a porous material having a particle size of 0.1 to 3 mm., said porous material being selected from the group consist-

ing of semi-coke, coke and graphite, and 10 to 25 percent by weight of a binder which secures said metal particles and said porous material particles together in a briquette.

5 2. An agent as claimed in claim 1, in which said selected metal is magnesium.

3. An agent as claimed in claim 1, in which said binder is selected from the group consisting of coal tar, coal tar pitch, petrochemical pitch and petrochemical bitumen.

10 4. A method of producing an addition agent for inoculation of a molten metal bath, comprising admixing 5 to 50 parts by weight of a metal selected from the group consisting of alkali metal and alkaline earth metal having a particle size of 0.1 to 3 mm., 50 to 80 parts by weight of a porous material having a particle size of 0.1 to 3 mm., said porous material being selected from the group consisting of semi-coke, coke and graphite, and 10 to 25 parts by weight of a thermoplastic binder, at a temperature of 80° to 130°C., briquetting the mixture to form solid bodies thereof, and heating the briquettes at a temperature from about 150° to about 250°C. for a time from about 15 minutes to about 90 minutes.

15 5. A process as claimed in claim 4, and further heating the briquettes at a temperature from about 250° to about 900°C. for a time from about 15 minutes to about 90 minutes.

20 6. A process as claimed in claim 4, in which said metal is magnesium.

25 7. A process as claimed in claim 4, in which said binder is selected from the group consisting of coal tar, coal tar pitch, petrochemical pitch and petrochemical bitumen.

\* \* \* \* \*